



US005547610A

# United States Patent [19]

Mortensen

[11] Patent Number: 5,547,610

[45] Date of Patent: Aug. 20, 1996

[54] CONDUCTIVE POLYMERIC ADHESIVE FOR FLOORING CONTAINING SILVER-COATED NON-CONDUCTIVE FIBER CORES

[75] Inventor: Kelly J. Mortensen, Conyngham, Pa.

[73] Assignee: Forbo Industries, Inc., Hazelton, Pa.

[21] Appl. No.: 237,026

[22] Filed: May 3, 1994

[51] Int. Cl.<sup>6</sup> H01B 1/16; D02G 3/00

[52] U.S. Cl. 252/514; 264/104; 524/457; 428/378; 428/389

[58] Field of Search 252/512, 514; 264/104; 524/457; 428/378, 389

## [56] References Cited

### U.S. PATENT DOCUMENTS

|           |         |                  |           |
|-----------|---------|------------------|-----------|
| 3,877,965 | 4/1975  | Broadbent et al. | 427/304   |
| 4,042,737 | 8/1977  | Forsgren et al.  | 428/96    |
| 4,247,596 | 1/1981  | Yee              | 428/380   |
| 4,534,886 | 8/1985  | Kraus et al.     | 252/502   |
| 4,566,990 | 1/1986  | Lim et al.       | 252/503   |
| 4,729,809 | 3/1988  | Dery et al.      | 156/306.6 |
| 4,752,415 | 6/1988  | Iwaskow et al.   | 252/511   |
| 4,882,089 | 11/1989 | Iwaskow et al.   | 428/242   |
| 5,075,038 | 12/1991 | Cole et al.      | 252/514   |
| 5,229,037 | 7/1993  | Nakano et al.    | 252/512   |
| 5,262,229 | 11/1993 | Lampert et al.   | 428/220   |
| 5,286,417 | 2/1994  | Mahmoud et al.   | 252/518   |
| 5,378,407 | 1/1995  | Chandler et al.  | 252/518   |

### OTHER PUBLICATIONS

S. M. Darwish, A. Niazi, A. Ghania, M. E. Kassem; Improving the Electrical Properties of Structural Epoxy Resin Adhesives; Jan. 1991.

Int. J. Adhesion and Adhesives; International News, p. 7; Electrically Conductive Epoxy, Jan. 1982.

Adhesive Abstracts, May 1988, p. 11; EMI/RFI Conductive Adhesives; EMI/RFI Conductive Caulking and Adhesives.

Adhesives Abstracts, May 1989, p. 9; TRA-Shield 2867; Conductive Silver Epoxy Coating.

Adhesives Abstracts, Sep. 1989, pp. 9-10; B-568 UV Curing Conductive Adhesive.

Adhesives Age, Apr. 1990, p. 8; Solvent Free Epoxy Series.

DIALOG FILE 399:CA Search; American Chemical Society; 113025206 CA: 113(4)25206M Journal Electroconductive Glue Line by Metalized Carrier 1989 no month available.

Primary Examiner—Paul Lieberman

Assistant Examiner—M. Kopec

Attorney, Agent, or Firm—R. Anthony Diehl; William H. Murray

## [57] ABSTRACT

Compositions, methods of providing compositions, flooring assemblies incorporating compositions, and methods for discharging accumulated electrostatic charges utilizing compositions of conductive adhesive are provided. The compositions comprise a non-conductive adhesive in which a plurality of silver plated or coated conductive fibers are dispersed such that the conductive fibers form an electroconductive chain when applied to a substrate.

12 Claims, 3 Drawing Sheets





*FIG. 1*



*FIG. 2*



*FIG. 2A*



FIG. 3



*FIG. 4*



*FIG. 4A*

**CONDUCTIVE POLYMERIC ADHESIVE FOR  
FLOORING CONTAINING SILVER-COATED  
NON-CONDUCTIVE FIBER CORES**

**FIELD OF INVENTION**

This invention relates to a conductive adhesive composition for flooring and, in particular, to a conductive adhesive composition comprised of a non-conductive adhesive and conductive fibers.

**BACKGROUND OF THE INVENTION**

Electrostatic discharge is problematic in the manufacturing, assembling, and functioning of parts for various electrical and electronic equipment, particularly semiconductor devices. More specifically, burn damage to the parts produced or assembled may result from the discharge of accumulated electrostatic charges within a room. Further, electrostatic charging of a room may result in adherence of dust to room surfaces. Finally, electrostatic discharge may cause electrical and electronic equipment to malfunction. Thus, the surfaces, i. e., walls, ceilings, and floors, of rooms in which electrical and electronic parts are manufactured and in which electronic equipment is utilized ideally are electroconductive so that any electrostatic charges within the room can be leaked to prevent the charging of the room.

Because electrostatic charges may accumulate on the conductive flooring utilized in such rooms, it is desirable to provide a means for discharging the accumulated charges from the conductive flooring material. Conductive flooring adhesives, which provide electroconductivity between the flooring and a conductor, such as a ground strap or wire, are commonly used for this purpose. Generally, the conductive adhesives are either non-conductive adhesives containing carbon fibers or conductive epoxies.

Utilization of these conventional adhesives is problematic for a variety of reasons. The application of carbon fiber or carbon coated fiber containing conductive adhesives is a labor intensive process because use of these adhesives may require the application of a conductive primer. Additionally, the carbon or carbon coated fibers within the adhesive lose their conductivity over time, possibly due to the cracking or breaking of the fibers. For those adhesives in which conductive epoxies are used, on-site mixing of the components of the epoxy is required which is a labor intensive process.

**SUMMARY OF THE INVENTION**

The present invention provides compositions, methods of providing compositions, flooring assemblies incorporating compositions, and methods for discharging accumulated electrostatic charges utilizing compositions of conductive adhesive that are cost-effective, durable, and easily applied. Such compositions comprise a non-conductive adhesive and a plurality of conductive fibers dispersed within the non-conductive adhesive, the amount and dimensions of the conductive fibers such that the conductive fibers form an electroconductive chain when the composition is applied to a substrate. By adhering conductive flooring material to the composition of the present invention and establishing an electrical connection between the adhesive, the flooring material, and ground, electrical charges may be discharged from the conductive flooring material.

The conductive adhesive composition of the present invention comprises:

- (a) a non-conductive adhesive; and

(b) a plurality of conductive fibers dispersed within the non-conductive adhesive in an amount effective to form an unbroken electroconductive chain when the conductive adhesive composition is applied to a substrate, the non-conductive fibers comprising non-conductive fiber cores plated or coated with silver.

The invention further provides a method for providing a conductive adhesive composition comprising mixing into a non-conductive adhesive a plurality of conductive fibers in an amount effective to form an unbroken electroconductive chain when the conductive adhesive composition is applied to a substrate, the plurality of conductive fibers comprising non-conductive fiber cores plated or coated with silver.

Further, the invention provides an electrically conductive assembly for floors, comprising:

- (a) a conductive adhesive composition comprising a plurality of conductive fibers dispersed within a non-conductive adhesive in an amount effective to form an electroconductive chain when the conductive adhesive composition is applied to a substrate, the plurality of conductive fibers comprising non-conductive fiber cores plated or coated with silver;
- (b) a conductive flooring material adhered to and on the conductive adhesive composition; and
- (c) a conductor in electrical contact with the electroconductive chain of the conductive adhesive composition and the conductive flooring.

Finally, the present invention provides a method for discharging electrical charges from a conductive flooring material, comprising the steps of:

- (a) applying a conductive adhesive composition to a substrate, the conductive adhesive composition comprising a plurality of conductive fibers dispersed within a non-conductive adhesive in an amount effective to form an unbroken electroconductive chain when the conductive adhesive composition is applied to a substrate, the plurality of conductive fibers comprising non-conductive fiber cores plated or coated with silver, each of the plurality of conductive fibers having a length of about 200 mils and a diameter of about 1.8 denier;
- (b) adhering a conductive flooring material to and on the conductive adhesive; and
- (c) establishing an electrical connection among the fibers of the conductive adhesive, the conductive flooring material, and a ground.

**BRIEF DESCRIPTION OF THE DRAWINGS**

FIG. 1 is an enlarged cross-sectional view of a conductive fiber for use in the subject invention.

FIG. 2 is a perspective view of the conductive adhesive composition of the subject invention applied to a substrate.

FIG. 2a is a magnified detailed plan view of the conductive adhesive composition of the subject invention applied to a substrate.

FIG. 3 is a perspective view of flooring tiles adhered to the conductive adhesive composition applied to a substrate.

FIG. 4 is a plan view of the trowel utilized to apply the conductive adhesive composition of the present invention.

FIG. 4a is a magnified plan view of a trowel tooth illustrating the dimensions of the teeth of the trowel depicted in FIG. 4.

**DESCRIPTION OF THE PREFERRED  
EMBODIMENTS**

Referring to FIG. 2, the conductive adhesive composition 16 of the present invention comprises flexible conductive

fibers **10** dispersed within a non-conductive adhesive **18** to form an unbroken electroconductive chain, i.e., so that substantially every fiber **10** is in contact, directly or indirectly with substantially all fibers **10**.

The conductive fiber **10** for use in the subject invention is shown in FIG. 1. The conductive fiber **10** comprises a non-conductive fiber core **12** and at least one layer of adherent conductive material **14** on the non-conductive fiber core **12**. The non-conductive fiber core **12** may be formed from cellulose, cotton, silk, wool, nylon, polyester, acrylic, or the like. The non-conductive fiber core is preferably flexible. The type of material from which the non-conductive fiber core **12** is formed will be determined by the processing properties and the end-use desired for the conductive adhesive composition **16**. It is preferred that the non-conductive fiber core **12** is formed from nylon because of the heat resistance properties and strength of nylon.

The non-conductive fiber core **12** is plated or coated with a conductive material **14** such as a metal, carbon, or the like. Plating of the non-conductive fiber core **12** can be accomplished by any of the conventional plating methods. Preferably, the non-conductive fiber core **12** is coated with silver. Suitable silver coated nylon fibers are available from Sauquoit Industries, Inc., Scranton, Pa. The silver coated nylon fibers are made, in general, by the procedures described in U.S. Pat. No. 3,877,965 which is incorporated herein, in its entirety, by reference.

The conductive adhesive composition **16** of the present invention is prepared by mixing the conductive fibers **10** with the non-conductive adhesive **18**. The non-conductive adhesive **18** of the present invention may be any of the conventional flooring adhesives. Exemplary adhesives include, without limitation, acrylic adhesives, latex adhesives, and rubber adhesives such as styrene-butadiene rubber adhesive.

Typically the conventional conductive flooring that is utilized is such that an acrylic adhesive will be preferred for use as the non-conductive adhesive **18**. Exemplary acrylic adhesives include, without limitation, **531<sup>TM</sup>**, a water-based acrylic adhesive, and **421<sup>TM</sup>**, a solvent-based acrylic adhesive, both of which are commercially available from Eurocol b.v.

The amount of the conductive fibers **10** added to the non-conductive adhesive **18** must be carefully regulated. The addition of too great an amount of fiber may render the conductive adhesive composition **16** difficult to process and spread by trowel and may affect the composition's adhesive properties. If an insufficient amount of conductive fibers is added, the conductive properties of the conductive adhesive composition **16** will be affected in that the amount of the conductive fibers **10** will not permit the formation of an unbroken electroconductive chain so that each fiber in the composition is in contact with every other fiber in the composition as depicted in FIG. 2a. Preferably, an amount of about 58 grams of the conductive fibers **10** are added per gallon of the non-conductive adhesive **18**.

The length of the conductive fibers **10** utilized is important also. As is shown in FIG. 2a, the conductive fibers **10** must touch to form a conductive chain. If the conductive fibers **10** are too short, they will not touch to form an unbroken conductive chain, as depicted in FIG. 2a, when the adhesive composition **16** of the present invention is spread onto a substrate **20**. If the conductive fibers **10** are too long, they will curl so as not to form a contiguous chain. Additionally, fibers that are too long will be very difficult to trowel. Preferably, the conductive fibers **10** each have a length of about 200 mils.

The diameter of the conductive fibers **10** is not critical to the practice of the invention. However, smaller diameter fibers are preferred because they can provide adequate conductivity at a lower cost when compared with larger diameter fibers. The conductive fibers **10** preferably have a diameter of about 1.8 denier.

The conductive adhesive composition **16** of the present invention must be applied to the substrate **20** by use of the trowel **26**, depicted in FIG. 4. The trowel **26** is generally planar and rectangular and has teeth **28** projecting from one edge thereof with spaces **30** therebetween. The trowel is designed so that the conductive adhesive composition **16** may be spread onto the substrate in parallel rows of a height determined by the configuration of the spaces **30**. Further, the configuration of the teeth **28** and the spaces **30** are such that the parallel rows of the adhesive composition **16** are in sufficient proximity so that the conductive fibers **10** will overlap the parallel rows of the adhesive composition **16** so as to form an unbroken electroconductive chain. The spaces of the trowel are additionally configured to permit the conductive fibers **10** to flow through the spaces **30** as the conductive adhesive composition **16** is spread onto the substrate **20**. This flow provides for the orientation of the conductive fibers **10** along the plane of the top surface of the substrate **20** in which trowel **26** moves.

Specifically, each of the teeth **28** ends in a point. Near the point, each tooth **28** has angled straight edges, the angle being small so that the sides of the rows of conductive adhesive composition **16** will be close together. The edge of trowel **26** intermediate each pair of the teeth is smoothly curved inward, without internal corners, to prevent bunching of conductive fibers **10** and so that each row of the conductive adhesive composition **16** has a convex upper surface. Trowel **26** may be formed from any conventional trowel material. Preferably trowel **26** is formed from steel.

FIG. 3 illustrates an electrically conductive assembly **40** for floors. In this assembly the conductive adhesive composition **16** is used to bind the conductive flooring material **24** to a substrate **20**. Electrical continuity among the conductive adhesive **16**, the conductive flooring material **24**, and a ground may be provided by any conductor conventionally used for establishing such continuity. As depicted in FIG. 3, electrical continuity may be provided by a ground strap **22**.

After troweling of the layer of the adhesive composition **16** onto the substrate **20**, the ground strap **22** is placed on the adhesive composition **16**. The conductive flooring material **24** is then applied on top of the adhesive composition **16** and the ground strap **22**. The conductive flooring material **24** is preferably in the form of tiles, which may be, for example **COLOREX<sup>TM</sup>** tiles as available from Forbo Industries, Inc. or any commercially available conductive tiles. The ground strap **22** is placed on the conductive adhesive **16** so as to contact the conductive fibers **10** as well as the conductive flooring tiles **24** in order to establish an electrical flow path.

It is well known to provide electrical continuity between prior art conductive adhesives for flooring, conductive flooring tiles, and a ground by a variety of conductors. For example, metal plated ground straps, including copper ground straps, may be used as conductors by embedding the ground straps into a conductive adhesive underlying conductive flooring tiles and connecting the ground straps to a grounding means. However, conventional metal plated ground straps are difficult to handle and subsequent corrosion of the straps can interfere with the electrical continuity.

Silver coated nylon fabric ground straps **22** have been found to provide a less expensive, easier to handle alterna-

tive conductor. Further, as the silver corrodes, electrical conductivity is retained because silver corrosion does not create an insulating effect. In the present invention, therefore, silver coated nylon fabric ground straps are the preferred conductors for providing electrical continuity among the conductive fibers 10, the conductive adhesive composition 16, and the conductive flooring tiles 24 and a grounding means. In general, one three foot length of ground strap for every 500 square feet of flooring is sufficient.

It is thought that the conductive adhesive composition of the present invention and many of its advantages will be understood from the foregoing description. It will be apparent that various changes may be made without departing from the spirit or the scope of the invention or sacrificing all of its material advantages. The invention has been described herein for the purpose of illustration and it is not to be construed or limited thereby, but it is intended to cover all changes and modifications within the spirit and scope thereof.

What is claimed is:

1. A conductive adhesive composition, comprising:
  - (a) a non-conductive Polymeric adhesive; and
  - (b) a plurality of conductive fibers dispersed within the non-conductive adhesive in an amount effective to form an unbroken electroconductive chain when the conductive adhesive composition is applied to a substrate, the conductive fibers comprising non-conductive fiber cores plated or coated with silver, wherein: the non-conductive fiber cores are selected from the group consisting of nylon, polyester, acrylic, cellulose, cotton, silk, or wool.
2. The composition of claim 1, wherein the amount of conductive fibers is about 58 g. per gallon of the non-conductive adhesive.

3. The composition of claim 1, wherein each of the conductive fibers has a length of about 200 mils.

4. The composition of claim 1, wherein each of the conductive fibers has a diameter of about 1.8 denier.

5. The composition of claim 1, wherein the non-conductive adhesive is an acrylic adhesive.

6. The composition of claim 1, wherein the non-conductive adhesive is a latex adhesive.

7. The composition of claim 1, wherein the non-conductive adhesive is a rubber adhesive.

8. The composition of claim 1, wherein each of the conductive fibers has a length of about 200 mils and a diameter of about 1.8 denier and the amount of conductive fibers is about 58 g. per gallon of the non-conductive adhesive.

9. A method of providing a conductive adhesive composition, comprising the step of mixing into a non-conductive Polymeric adhesive a plurality of conductive fibers in an amount effective to form an unbroken electroconductive chain when the conductive adhesive composition is applied to a substrate, the plurality of conductive fibers comprising non-conductive fiber cores plated or coated with silver, wherein the non-conductive fiber cores are selected from the group consisting of nylon, polyester, acrylic, cellulose, cotton, silk, or wool.

10. The method of claim 9, wherein the amount of conductive fibers is about 58 g. per gallon of the non-conductive adhesive.

11. The method of claim 9, wherein each of the conductive fibers has a length of about 200 mils.

12. The method of claim 9, wherein each of the conductive fibers has a diameter of about 1.8 denier.

\* \* \* \* \*